

## UNITED STATES PATENT OFFICE

2,156,626

PHOTOGRAPHIC DEVELOPING MEDIUM  
PRODUCING FINE GRAIN RESULTSGarnet P. Ham, Old Greenwich, Conn., assignor  
to American Cyanamid Company, New York,  
N. Y., a corporation of MaineNo Drawing. Application March 16, 1938,  
Serial No. 196,157

10 Claims. (Cl. 95—88)

This invention relates to a photographic developer and more particularly, to a developer capable of giving a fine grain.

The necessity of great enlargement which is 5 increasingly important with the advance of the miniature camera and also the need for motion picture positive film has made it necessary to depart from some of the standard developers used in the development of films where great 10 enlargement and hence extreme fine grain was not necessary. This has resulted in the development of innumerable fine grain developers in the past two years. These developers have followed along three main lines.

15 One class of developer using the standard Metol and hydroquinone with very low alkalinity given by borax or similar weak alkalies used in small quantities does not sacrifice the speed of emulsion to any serious extent but results in a grain 20 which, while finer than those produced by standard developers, leaves much to be desired in the case of finer grain films.

25 The second class of developers is represented by those using p-phenylenediamine as their base with or without Glycine and small amounts of Metol. This class of developers gives an extremely fine grain but at the expense of contrast and particularly, of emulsion speed. In other words, greatly increased exposure is necessary.

30 A third class of fine grain developers is represented by the so-called physical developers in which colloidal silver is plated out onto a latent image on the film. This type of developer with suitable skilled operation is capable of giving a fine grain but is more difficult to use than those depending on chemical action.

35 It has been proposed recently to combine chemical developers with physical developers. This is frequently referred to in the art as silver loading a developer and among the most successful 40 compromise developers of this type is the well-known Champlin #15 having the following formula in which the parts are by weight except in the cases of the water and the isopropyl alcohol 45 where the corresponding volumes are given:

|                              | Parts |
|------------------------------|-------|
| Water                        | 1000  |
| Rubinol or pyro              | 3.5   |
| Sodium sulphite              | 60.0  |
| 50 Acid benzoic              | 1.2   |
| Acid salicylic               | 0.5   |
| Acid boric                   | 2.5   |
| Acid digallic (tannic)       | 1.0   |
| 55 Glycin                    | 11.5  |
| Paraphenylenediamine         | 11.5  |
| Alcohol iso propyl 97%       | 50.0  |
| Nickel and ammonium sulphate | 1.0   |

60 The best of the fine grain developers produced heretofore produce a grain which is satisfactory

for most uses but they are subject to certain disadvantages. The p-phenylenediamine developers as noted above require a greatly increased exposure with high speed panchromatic films and as these films are being increasingly used because of their high speed, this disadvantage is extremely serious. Most fine grain developers, even those of the Metol-hydroquinone type, likewise require for the production of real fine grain a considerable underdevelopment so that the resulting negatives are of relatively low contrast, a gamma of about 0.7 being often recommended with these developers. This is a serious disadvantage in the case of many negatives because in order to compensate for the 15 low contrast of the developed negative it is necessary to use printing papers of excessive contrast and as is well known, the emulsion character and general tone and gradation of high contrast papers are not as desirable as those 20 of softer papers.

According to the present invention, a developer of the combined chemical and physical type is produced which gives a grain as fine and in some cases finer than the best obtainable with the fine grain developers known at the present time without possessing their disadvantages. The developer of the present invention does not reduce the emulsion speed; in fact, as compared to the best of the compromise fine grain developers on 30 the market at the present time, it shows a slight increase in emulsion speed amounting to from 20-30%. Another important advantage of the present developer is that it is not necessary in order to obtain fine grain to underdevelop the 35 negative producing a flat negative of excessively low contrast. On the contrary, the developing time can be increased to produce a negative of 40 normal contrast (when compared with negatives developed in standard developers which are not fine grain) without loss of the fine grain. This is an important advantage because extreme fineness of grain has been accorded an importance entirely out of proportion to the real facts. Standard fine grain developers now available 45 will give a sufficiently fine grain even with fast panchromatic film such as the standard Eastman Super X to permit enlargement to adequate size for 99% of the work actually undertaken. The other factors such as contrast of the negative, 50 emulsion speed and the like are in many, if not most, cases more important. It is an outstanding advantage of the present invention that the developer meets all of the requirements and does not compromise with speed or quality.

55 A developer of the present invention consists in a chemical developer which may be of various formulation but preferably a p-phenylene diamine base developer to which sufficient Metol has been added for adequate shadow detail,

standard preservative such as sodium sulfite, buffers and alkali combined with colloidal silver or silver compounds stabilized with a protective colloid. To obtain the full results, the developer 5 should also be activated by exposure to actinic light.

I have found that it is not necessary to use an extremely narrow range of proportions of chemical developers. The choice of protective 10 colloid is also very wide. Gelatin, alkyl cellulose, water-soluble polyvinyl alcohol and many other colloids can be used provided, of course, that the colloid does not react with the chemical components of the developer. The activated silver 15 chloride is prevented from precipitation by the colloid and apparently plates out on the latent image as the latter is formed by the action of the chemical developers. The appearance of the negative closely resembles that obtained by a 20 true physical developer but the action and the time of development correspond to that of a chemical developer of the character represented by the chemical constituents of the developer of the present invention. I believe that the fineness 25 of grain without sacrifice of emulsion speed is in large measure due to the fact that the physical development is kept in proportion to the chemical development by the presence of the colloid which prevents premature decomposition of the 30 silver halide in the developer. The present invention is, however, not intended to be limited to any theory of action.

The developer of the present invention possesses an extraordinary stability both of high 35 temperatures and to very low temperatures. Thus, for example, tests with the developer which is described in the specific examples below were made at 120° F., the temperature frequently reached in the mail rooms of steamers in the 40 tropics. After thirty days at 120° F., the developer showed but little precipitate and its developing action was almost indistinguishable from that of fresh developer. A month's storage in a refrigerator at a temperature only a little above 45 freezing showed no noticeable effect. Under similar treatment, Champlin #15 showed marked decomposition at 120° F. and when used for developing films gave a lower range of detail and showed a markedly decreased speed, that is to say, an 50 exposure of almost double was required with Super X in order to obtain the same results.

A further important advantage of the developer of the present invention lies in the fact that it is relatively insensitive to temperature. Development 55 can be carried out at 70° F. or even materially higher (with, of course, a corresponding shortening of developing time) without any noticeable loss of fineness of grain or contrast in the negative.

The developer of the present invention gives 60 excellent results with all kinds of film including slow and fast panchromatic, orthochromatic, motion picture positive and other negative material. The advantages of maintenance of emulsion speed 65 are particularly noticeable with fast panchromatic films. As is well-known, there is comparatively little decrease in emulsion speed with the usual fine grain developer in the case of slow speed, ultrafinegrain panchromatic film and the high inherent contrast of this type of material makes 70 the underdevelopment required by the usual fine grain developer relatively unobjectionable. It is an advantage of the present invention that the developer is useful for all of the ordinary types 75 of negative material even though its greatest

advantages over known developers are to be found when it is used with high speed panchromatic film.

The invention will be described in conjunction with specific examples setting out formulae which I have found to be the best all round formulae 5 for use with panchromatic film. The invention is not limited to the details of these particular formulae and the components can be varied within wide limits while retaining the advantages of 10 the present invention.

#### Example 1

A solution is prepared having the following composition:

|                      | Parts |
|----------------------|-------|
| Paraphenylenediamine | 5.7   |
| Metol                | 1.5   |
| Glycin               | 5.7   |
| Sodium sulphite      | 34.0  |
| Boric acid           | 1.3   |
| Salicylic acid       | 0.2   |
| Benzoic acid         | 1.02  |
| Water to make        | 500.0 |

A second solution is prepared having the following composition:

|                    | Parts   |
|--------------------|---------|
| Potassium chloride | 0.25    |
| Egg albumen        | 0.1-0.5 |
| Silver nitrate     | 0.25    |
| Water              | 100.00  |

The silver chloride formed in this solution is prevented from precipitating by the colloidal albumen present. The mixture is then activated by 35 actinic light for a period of time varying from 5 to 15 minutes or even longer depending on the volume of the solution treated, the intensity of the light, etc. The time is not critical and longer activation does no harm. After activation is 40 complete, the solution is added to the first solution and the mixture is permitted to ripen for from 1 to 8 hours at ordinary room temperature, preferably in the absence of strong actinic light. At the end of this period, a certain amount of 45 silver coagulate will be noted and this is filtered off. The remaining clear solution, which is very light amber in color, is bottled and constitutes the finished product which is used at full strength.

The final solution is thoroughly light stable and does not have to be stored in dark bottles. It keeps for months and can be used repeatedly. Thus, for example, a pint of developer can be used to develop from 6 to 10 standard thirty-six 55 exposure rolls of 35 mm. film without any noticeable loss in quality of the negative. Care, of course, is taken to increase the developing time with each roll. This represents a considerably longer life than any of the standard fine grain 60 developers at present available.

Development is preferably effected at ordinary room temperature of about 70° F. but satisfactory results can be obtained at 65° F. and higher temperatures can also be used. The development 65 time will vary with different films; for example, satisfactory contrast for use with the ordinary grades of paper on fast panchromatic film such as Eastman Super X is obtained by developing at 70° F. for 18 to 25 minutes in fresh developer 70 depending on the degree of agitation. There is no tendency to deposit stains on the film and completely stagnant development can therefore be used which is an added convenience where facilities for continuous agitation are lacking. Slow 75

panchromatic film of the type marketed by Eastman Kodak as Panatomic, by Du Pont as Micropan and by the Agfa Ansco Company as Finopan require shorter development time.

I have not determined just what takes place during activation of the silver halide and after addition to the chemical developing solution and the present invention is not limited to any theory of action. However, I believe that it is probable that far-reaching photo-activation of the silver halide takes place because there is some precipitate during activation in spite of the presence of the protective colloid. When the two solutions are mixed, some of the activated silver halide reacts with the chemical developing agents as there is a considerable precipitation of silver. I believe that this action proceeds only to the point at which the most strongly activated silver halide particles are attacked. During development there is a marked plating out of silver on the image as it forms by the action of the chemical developing agents and I believe that the activated silver halide or in some cases colloidal silver kept from precipitating by the protective colloid tends to plate out on the developing image with great rapidity. The plating action takes place much faster than with a pure physical developer.

As has been stated above, the egg albumen is merely representative of a number of protective colloids which appear to act because of their colloidal properties. Albumen gives very satisfactory results and is the preferred colloid but other colloids can be used. The proportions of the chemicals may be varied within wide limits and other chemical developing agents such as hydroquinone may be included.

#### Example 2

Two solutions are prepared as in Example 1 but water-soluble methyl cellulose is substituted for the egg albumen. The solutions are then mixed and subjected to activation with actinic light for from five to fifteen minutes or longer, followed by ripening at room temperature for from one to eight hours and filtering off the silver coagulate formed. The solution is of substantially the same light color as that of the first example.

The procedure described above in which mixing the solutions precedes light activation is simpler and gives results which are indistinguishable from those produced by separately activating the silver halide solution before mixing.

The developer does not appear to be extremely sensitive to slight changes in pH. However, the presence of buffers and preservatives for the colloid are desirable.

The production of activated silver halide solution can use various alkali metal chlorides or iodides. The potassium chloride of the examples gives excellent results but satisfactory results are obtainable with the iodide or with the chloride or iodide of sodium. The bromide is less desirable as it forms a silver compound which is excessively activated resulting in a loss of a large portion of the silver by precipitation. Mixtures of the alkali halides may also be used and if the amount of bromide present is small, such mixtures even though containing bromide give satisfactory results.

#### What I claim is:

1. A photographic developer comprising an aqueous dispersion containing unoxidized metal a colloidal silver halide and a protective colloid.
2. A photographic developer comprising an

aqueous dispersion containing unoxidized metal a colloidal light-activated silver halide and a protective colloid.

3. A photographic developer comprising an aqueous dispersion containing p-phenylenediamine, Glycine and Metol, preservatives, colloidal light-activated silver halide and a protective colloid.

4. A photographic developer comprising an aqueous dispersion containing p-phenylenediamine, Glycine and Metol, preservatives, colloidal light-activated silver halide and albumen.

5. A method of producing a photographic developer which comprises forming an aqueous dispersion of an alkali metal halide, a protective colloid and silver nitrate, subjecting the dispersion to the action of actinic light, adding to the dispersion an aqueous solution of organic chemical developing agents and at least one preservative, permitting the mixture to stand until precipitation has substantially ceased and removing the precipitate by filtration, the amount of organic chemical developing agents being largely in excess of that capable of reacting with the silver halide formed so that the dispersion contains unoxidized organic chemical developer.

6. A method of producing a photographic developer which comprises forming an aqueous dispersion of an alkali metal halide, a protective colloid and silver nitrate, subjecting the dispersion to the action of actinic light, adding to the dispersion a solution containing p-phenylenediamine, Glycine and Metol, permitting the mixture to stand until precipitation has substantially ceased and removing the precipitate by filtration, the amount of paraphenylenediamine, Glycine and Metol being largely in excess of that capable of reacting with the silver halide formed so that the dispersion contains unoxidized paraphenylenediamine, Glycine and Metol.

7. A method of producing a photographic developer which comprises forming an aqueous dispersion of an alkali metal halide, albumen and silver nitrate, subjecting the dispersion to the action of actinic light, adding to the dispersion a solution containing p-phenylenediamine, Glycine and Metol, permitting the mixture to stand until precipitation has substantially ceased and removing the precipitate by filtration, the amount of paraphenylenediamine, Glycine and Metol being largely in excess of that capable of reacting with the silver halide formed so that the dispersion contains unoxidized paraphenylenediamine, Glycine and Metol.

8. A method of producing a photographic developer which comprises forming an aqueous dispersion of an alkali metal halide, a protective colloid and silver nitrate, adding this dispersion to an aqueous solution of chemical developing agents and preservatives, subjecting the mixture to the action of actinic light, permitting the activated mixture to stand until precipitation has substantially ceased and removing the precipitate by filtration, the amount of organic chemical developing agents being largely in excess of that capable of reacting with the silver halide formed so that the dispersion contains unoxidized organic chemical developer.

9. A method of producing a photographic developer which comprises forming an aqueous dispersion of an alkali metal halide, a protective colloid and silver nitrate, adding this dispersion to an aqueous solution containing p-phenylenediamine, Glycine and Metol and preservatives, subjecting the mixture to the action of actinic

5 light, permitting the activated mixture to stand until precipitation has substantially ceased and removing the precipitate by filtration, the amount of paraphenylenediamine, Glycine and Metol being largely in excess of that capable of reacting with the silver halide formed so that the dispersion contains unoxidized paraphenylenediamine, Glycine and Metol.

10 10. A method of producing a photographic developer which comprises forming an aqueous dispersion of an alkali metal halide, albumen and silver nitrate, adding this dispersion to an aque-

ous solution containing p-phenylenediamine, Glycine and Metol and preservatives, subjecting the mixture to the action of actinic light, permitting the activated mixture to stand until precipitation has substantially ceased and removing the precipitate by filtration, the amount of paraphenylenediamine, Glycine and Metol being largely in excess of that capable of reacting with the silver halide formed so that the dispersion contains unoxidized paraphenylenediamine, Glycine and Metol. 5 10

GARNET P. HAM.

CERTIFICATE OF CORRECTION.

Patent No. 2,156,626.

May 2, 1939.

GARNET P. HAM.

It is hereby certified that error appears in the printed specification of the above numbered patent requiring correction as follows: Page 3, first column, line 73, and second column, line 1, claims 1 and 2 respectively, for "metal" read Metol,; and that the said Letters Patent should be read with this correction therein that the same may conform to the record of the case in the Patent Office.

Signed and sealed this 30th day of May, A. D. 1939.

(Seal)

Henry Van Arsdale  
Acting Commissioner of Patents.

5 light, permitting the activated mixture to stand until precipitation has substantially ceased and removing the precipitate by filtration, the amount of paraphenylenediamine, Glycine and Metol being largely in excess of that capable of reacting with the silver halide formed so that the dispersion contains unoxidized paraphenylenediamine, Glycine and Metol.

10 10. A method of producing a photographic developer which comprises forming an aqueous dispersion of an alkali metal halide, albumen and silver nitrate, adding this dispersion to an aque-

ous solution containing p-phenylenediamine, Glycine and Metol and preservatives, subjecting the mixture to the action of actinic light, permitting the activated mixture to stand until precipitation has substantially ceased and removing the precipitate by filtration, the amount of paraphenylenediamine, Glycine and Metol being largely in excess of that capable of reacting with the silver halide formed so that the dispersion contains unoxidized paraphenylenediamine, Glycine and Metol.

5

10

GARNET P. HAM.

## CERTIFICATE OF CORRECTION.

Patent No. 2,156,626.

May 2, 1939.

GARNET P. HAM.

It is hereby certified that error appears in the printed specification of the above numbered patent requiring correction as follows: Page 3, first column, line 73, and second column, line 1, claims 1 and 2 respectively, for "metal" read Metol,; and that the said Letters Patent should be read with this correction therein that the same may conform to the record of the case in the Patent Office.

Signed and sealed this 30th day of May, A. D. 1939.

(Seal)

Henry Van Arsdale  
Acting Commissioner of Patents.